

## UNITED STATES PATENT OFFICE

2,418,955

PROCESS OF REMOVING FOREIGN MATTER  
FROM MAGNESIUM SURFACES

Roy Shawcross, Salina, Pa., assignor to Aluminum Company of America, Pittsburgh, Pa., a corporation of Pennsylvania

No Drawing. Application May 25, 1943,  
Serial No. 488,403

2 Claims. (Cl. 252—136)

1

This invention relates to the treatment of magnesium surfaces to remove foreign matter therefrom. The contamination of magnesium surfaces by foreign materials may result from a number of causes. Such foreign materials are usually non-metallics included in or on the surface as the result of manufacturing operations, a common example being the carbonaceous deposit formed during the working of magnesium by the lubricant which is necessarily used in such working operations as rolling and drawing. The foreign material may firmly adhere to the metal surface or it may be imbedded therein. In many instances mere wiping or superficial abrasion of the surface will not remove these materials and a chemical treatment is necessary. The result of the chemical treatment may be to dissolve all or a part of the foreign material and to dissolve a film of magnesium, thus mechanically releasing and eliminating the foreign material. In any event, the use of such chemical treatment is beset with difficulties, particularly where large quantities of magnesium articles are handled. The chemical treatment if not closely controlled may remove too large an amount of the metal from the surface, it may etch or attack too deeply thus producing a rough surface, it may leave a dull surface of unsatisfactory appearance and it may secondarily stain the surface. To control the attack of the chemical and to produce a clean, smooth and relatively bright surface, the chemical treatment is often carried out at low temperatures or with comparatively small concentrations of the chemical with the result that the time of treatment is unduly extended.

An object of the invention is to provide a novel method of chemical treatment by which foreign materials may be satisfactorily removed from magnesium surfaces. Another object is to provide a chemical treatment by which this result may be accomplished in a relatively short time. Among further objects of the invention is the provision of a method of treatment which will produce a smooth, clean and relatively bright magnesium surface.

The invention is directed to the treatment of pure magnesium, magnesium of various grades of commercial purity and magnesium base alloys, such as those containing 70 per cent or more by weight of magnesium. The term "magnesium" as used herein and in the appended claims is intended to define and include all such grades and alloys as well as pure magnesium.

In accordance with this invention, the objects above described are obtained, in whole or in sub-

stantial part, by treatment of the magnesium surface with an aqueous solution containing an acid sulphate of sodium, potassium or ammonium (which elements are herein collectively referred to as alkali metals since ammonium quite often has the characteristics of such metals) or with an acidified aqueous solution of a sulphate selected from the group consisting of magnesium sulphate, aluminum sulphate and the double sulphates of alkali metal and aluminum, commonly referred to as alums. These compounds may be used singly or together. Usually I prefer the use of sodium acid sulphate since it gives excellent results and is cheap and plentiful but any of the others may be used with good results with the one exception that where iron is present in the solution the use of ammonium acid sulphate may, as hereinafter described, be disadvantageous if a clean surface without stains is desired. In practice the solution as used should contain about 5 per cent to about 25 per cent by weight of one of these compounds, or if two or more of the compounds are present that amount should represent the total present. Less than about 5 per cent by weight of one or a total of these compounds is not economical because treatment time is prolonged. At higher concentrations than 25 per cent the reaction is often too violent and unnecessary amounts of the treated metal are dissolved by the solution.

The process of obtaining a clean bright magnesium surface by the use of such solutions is often complicated by the presence of iron contamination in the solution, which contamination may be the result of the ordinary iron impurities in commercial grade chemicals, or the result of contamination of the solution during operations. In any event, the iron contamination will, in some cases, cause a staining of the sheet. On a bright clean surface this staining is undesirable although it in no way prevents the removal of foreign matter which is the primary object of the treatment. When magnesium sulphate, aluminum sulphate or an alum are substantial constituents of the treating solution, this iron staining seldom, if ever, occurs. But when the acid sulphates of the alkali metals are used alone, staining may be quite severe. This staining may be prevented, I have found, in whole or in substantial part by the addition of one or more of the following compounds; however, where ammonium acid sulphate is used, staining is not always eliminated or diminished:

The soluble sodium polyphosphates—such as  $(NaPO_3)_6$ , sometimes written  $Na_2P_6O_{18}$  and  $Na_6P_4O_{13}$ —in amount of about 0.2 per cent by

weight of the total solution. Increasing amounts are not harmful except as operating costs are increased, but generally I prefer to limit the amounts used to less than about 10 per cent by weight.

At least one of the aliphatic acids selected from the group consisting of acetic, tartaric and citric acids and used in total amount of not less than about 0.5 per cent by weight of the solution. Usually not more than about 15 per cent by weight of such an acid, or acids, is desirable because of the unnecessary cost involved in the use of further amounts.

At least one acid selected from the group consisting of tannic acid, gallic acid and pyrogallic acid used in amount of not less than 0.1 per cent nor more than about 5 per cent by weight of the solution.

Phosphoric acid used in amount of about 2 to about 5 per cent by weight of the total solution.

Solutions of the acid sulphates of alkali metals are sufficiently acid for the purposes of this invention, but solutions containing magnesium sulphate, aluminum sulphate or an alum must be acidified to an extent generally indicated by a ratio, in the treating solution, of one part of the salt to 0.8 part of sulphuric acid. I have found, however, that the sulphuric acid content of the solution may be as high as 15 per cent by weight. The method of treatment consists in contacting the magnesium surface with the acid sulphate or acidified sulphate solution, removing the surface from contact with the solution and allowing any solution remaining thereon to drain therefrom. If desired, the residual solution may be washed from the magnesium surface. Best results seem to be obtained when the solution is maintained at a temperature of about 60 to about 90° C. Lower temperatures may be maintained during operation with the result that the cleaning action proceeds at a slower rate. In many cases higher temperatures may result in too strong an attack and the dissolving of unnecessary amounts of metal from the surface undergoing treatment. The exact temperature to be used with any solution is readily determined in accordance with these principles by simple experiment. Similar principles may be applied to the time of immersion necessary for the best results. Usually 30 seconds to 3 minutes will give satisfactory commercial results.

The acid sulphates of the alkali metals, magnesium sulphate, aluminum sulphate or an alum may be used singly or in mixture. In the commercial operation of the process the solution is used over and over again and in time the reaction of the solution with the magnesium surfaces which are being treated will build up in the solution a content of magnesium sulphate. Also, under repeated reuse the reactants of the original solution are diminished by "drag out" as the magnesium articles are removed from the solution and by the reaction with the magnesium surface during treatment. However, this introduction into the treating solution of magnesium sulphate during continued use of the solution is a factor of which advantage may be taken. For instance, if one starts with a solution of sodium acid sulphate, the solution will, after repeated use, lose a material part of its sodium acid sulphate content, but at the same time it will gain in magnesium sulphate content until eventually the solution is composed largely of magnesium sulphate and sodium acid sulphate is no longer present in amounts necessary to the reaction.

In such a case it is possible to continue the use of the solution if, in accordance with this invention, the solution is from time to time fortified with sulphuric acid to maintain a ratio of free (i. e. uncombined) acid to magnesium sulphate as above mentioned or an excess of acid over that ratio. A substance such as one of the polyphosphates may have been used in the original acid sulphate solution to suppress the iron, but as the magnesium sulphate content of the solution builds up, the future use of the substance is no longer necessary since, as above described, iron staining rarely occurs in the presence of acidified magnesium sulphate.

It is possible, therefore, in the practice of the invention, to start with any one of the acid sulphates mentioned or with acidified solutions of aluminum sulphate or an alum and after the solution has been in use for some time to continue to practice the invention, without discarding the solution, by acidifying the solution to achieve the proper balance between the acid and the magnesium sulphate content acquired by the solution during treatment. Alternatively the solution may merely be discarded as the reaction and drag out diminish its reactive qualities. Again alternatively, the starting solution may be an acidified solution of magnesium sulphate, in which case after use it may be discarded or the acid balance between acid and magnesium sulphate maintained by the addition of sulphuric acid as the original acid content and magnesium sulphate content diminishes and the solution acquires additional quantities of magnesium sulphate as the result of the operations.

By the use of the methods of treatment above described, magnesium surfaces may be quickly and efficiently cleaned of foreign matter and a relatively smooth bright appearance achieved. The methods of this invention produce better results in commercial operations than those usually obtained by the use of acids as a cleansing medium.

As an example illustrative of the operation of the invention may be cited an instance where carbonized roll coating was removed from magnesium sheet. The sheet was treated for about 2 minutes in a solution containing 10 per cent by weight of  $\text{NaHSO}_4$  to which had been added 0.2 per cent by weight of  $(\text{NaPO}_3)_6$ . The solution was maintained at a temperature of about 158° F. Thereafter the sheet was removed from the solution and allowed to drain free of solution remaining on its surface. The result was a complete removal of the roll coating leaving a clean bright surface.

I claim:

1. The process of removing from a magnesium surface, roll coatings and similar foreign materials which comprises contacting the surface with an aqueous solution containing from about 5 to about 25 per cent by weight of an acid sulphate of an alkali metal and from about 0.2 to about 15 per cent by weight of a soluble sodium polyphosphate.

2. The process of removing foreign materials from magnesium surfaces which comprises contacting the surface with an aqueous solution containing in total amount from about 5 to about 25 per cent by weight of at least one of the sulphates selected from the group consisting of magnesium sulphate, aluminum sulphate and double sulphate of aluminum and alkali metal and also containing sulphuric acid in amount at least approximating a ratio of one part of said sulphate to 0.8 part

5

of said acid but not exceeding 15 per cent by weight of said acid.

ROY SHAWCROSS.

## REFERENCES CITED

The following references are of record in the file of this patent:

## UNITED STATES PATENTS

| Number    | Name    | Date          | 10 |
|-----------|---------|---------------|----|
| 1,918,545 | Hoy     | July 18, 1933 |    |
| 2,287,050 | Miller  | June 23, 1942 |    |
| 2,302,939 | De Long | Nov. 24, 1942 |    |

6

| Number    | Name    | Date           |
|-----------|---------|----------------|
| 2,092,913 | Fiske   | Sept. 14, 1937 |
| 1,795,473 | Burdick | Mar. 10, 1931  |
| 2,314,369 | Reed    | Mar. 23, 1943  |

## FOREIGN PATENTS

| Number  | Country | Date         |
|---------|---------|--------------|
| 500,009 | British | Feb. 1, 1939 |

## OTHER REFERENCES

Condensed Chemical Dictionary, 3rd ed., revised (1942) Reinhold Pub. Co., N. Y., page 586.  
(Copy in Div. 64.)